

## UNITED STATES PATENT OFFICE

2,054,927

## CORROSION RESISTANT ALLOY

Carl Carius, Essen, Germany, assignor to Fried.  
Krupp Aktiengesellschaft, Essen-on-the-Ruhr,  
Germany

No Drawing. Application June 28, 1935, Serial  
No. 28,943. In Germany September 13, 1934

3 Claims. (Cl. 75—125)

The invention relates to corrosion-resistant alloys and has more particularly reference to corrosion-resistant chromium-nickel-iron alloys which according to the invention further contain antimony. Alloys of this composition are distinguished by a very high resistance to corrosion and are in particular far superior to the usual chromium-nickel-molybdenum-iron alloys, for example to the known austenitic chromium-nickel-molybdenum steels, as to resistance to caustic soda lye or potash lye and in particular to hydrochloric acid. The invention further includes the improvement of alloys of this class by adding copper to them.

15 The alloys according to the invention may be composed about as follows:

|            | Percent  |
|------------|----------|
| Carbon     | 0 to 1   |
| Chromium   | 10 to 25 |
| 20 Nickel  | 20 to 40 |
| Molybdenum | 1 to 10  |
| Antimony   | 2 to 7   |
| Copper     | 0 to 10  |

25 and the remainder iron, without or with the normal impurities.

Alloys have been proved particularly advantageous which contain

|            | Percent       |
|------------|---------------|
| 30 Carbon  | less than 0.2 |
| Chromium   | 13 to 20      |
| Nickel     | 27 to 33      |
| Molybdenum | 2 to 5        |
| Antimony   | 3 to 5        |

35 and the remainder iron, without or with the normal impurities, and, under circumstances, further

|        | Percent |
|--------|---------|
| Copper | 2 to 6  |

40 An alloy, for example, containing

|               | Percent |
|---------------|---------|
| Carbon        | 0.15    |
| Chromium      | 18      |
| Nickel        | 30      |
| 45 Molybdenum | 5       |
| Antimony      | 5       |
| Copper        | 5       |

and the remainder iron, without or with the normal impurities, was not attacked to an extent

50 worth mentioning by 20% hot hydrochloric acid.

The following tables show the compositions of four iron alloys and their losses of weight in hydrochloric acid solutions of different concentrations and at different temperatures.

The dimensions of the castings tested were 60 x 20 x 8 mm.

## Analyses

| Symbol of the alloy | C    | Si   | Mn   | Cr   | Ni   | Mo   | Sb   | Cu  | 10 |
|---------------------|------|------|------|------|------|------|------|-----|----|
| I                   | 0.04 | 0.50 | 0.50 | 17.5 | 30.3 | 5.2  | 5.25 | 4.9 |    |
| II                  | 0.01 | 0.37 | 0.39 | 18.9 | 29.9 | 5.45 | 2.03 | 5.0 |    |
| III                 | 0.04 | 0.40 | 0.30 | 18.4 | 30.2 | 5.3  | —    | 5.1 |    |
| IV                  | 0.02 | 0.27 | 0.44 | 18.3 | 29.5 | 5.35 | —    | —   | 15 |

| Corrosive agent | Concen-<br>tration<br>in<br>percent | Temper-<br>atures in<br>°C. | Loss of weight of the<br>castings after 200 hour<br>test, in g/h/m <sup>2</sup> |      |      |      | 20 |
|-----------------|-------------------------------------|-----------------------------|---------------------------------------------------------------------------------|------|------|------|----|
|                 |                                     |                             | I                                                                               | II   | III  | IV   |    |
| HCl             | 10                                  | 40                          | 0.3                                                                             | 0.39 | 1.8  | 0.6  | 25 |
|                 |                                     | 60                          | 0.5                                                                             | 0.57 | 3.6  | 2.5  |    |
|                 |                                     | 80                          | 0.7                                                                             | 0.78 | 8.0  | 15.0 |    |
|                 |                                     | 40                          | 0.3                                                                             | 0.41 | 1.9  | 1.0  |    |
| HCl             | 15                                  | 60                          | 0.4                                                                             | 0.43 | 5.0  | 4.0  | 40 |
|                 |                                     | 80                          | 0.6                                                                             | 0.78 | 11.0 | 16.0 |    |
|                 |                                     | 40                          | 0.35                                                                            | 0.30 | 2.1  | 1.9  |    |
|                 |                                     | 60                          | 0.5                                                                             | 0.29 | 6.2  | 5.0  |    |
| HCl             | 20                                  | 80                          | 3.9                                                                             | 0.95 | 20.0 | 17.0 | 50 |
|                 |                                     | 40                          | 0.65                                                                            | 0.50 | 3.6  | 2.0  |    |
|                 |                                     | 60                          | 1.0                                                                             | 0.70 | 10.0 | 6.0  |    |
|                 |                                     | 80                          | 4.9                                                                             | 3.0  | 30.0 | 20.0 |    |

In order to impart to the alloys particularly good properties, they may be subjected to a heat treatment as usual with corrosion-resistant steels.

What I claim and desire to secure by Letters Patent is:—

1. An alloy of the class described and containing 0.02-1% carbon, 10-25% chromium, 20-40% nickel, 1-10% molybdenum, 2-7% antimony, 0.5-10% copper, and the remainder iron.

2. An alloy of the class described and containing 0.02-0.2% carbon, 13-20% chromium, 27-33% nickel, 2-5% molybdenum, 3-5% antimony, 2-6% copper, and the remainder iron.

3. An alloy of the class described and containing 0.15% carbon, 18% chromium, 30% nickel, 5% molybdenum, 5% antimony, 5% copper, and the remainder iron.

CARL CARIUS. 50